

# UNITED STATES PATENT OFFICE.

GILBERT S. DEAN, OF SAN FRANCISCO, CALIFORNIA.

## METHOD OF PREPARING NITRO-GLYCERINE COMPOUNDS.

SPECIFICATION forming part of Letters Patent No. 241,941, dated May 24, 1881.

Application filed July 29, 1879.

To all whom it may concern:

Be it known that I, GILBERT S. DEAN, of the city and county of San Francisco, State of California, have invented a new and useful Improvement in Explosive Compounds wherein Nitro-Glycerine is used, of which the following is a specification.

The object of the invention is to increase the safety of nitro-glycerine compounds.

10 I have found that water intimately mixed with nitro-glycerine diminishes its liability to explode, both in mass and in detail—the greater the quantity of water present the less the liability of producing an accidental explosion. The essential point of the present invention is, then, the conferring of additional safety upon nitro-glycerine by mixing with water. In order to produce such an intimate mixture it is necessary that the liquid mobility of the nitro-glycerine should be removed. This can be done, as is well known, by the addition of a pulverulent solid to the nitro-glycerine.

25 In order to remove the liquid form of the nitro-glycerine without substantial diminution of force I add thereto a nitro-compound of the cellulose group. Nitro-cellulose may be used, if in fine powder, but I prefer nitro-dextrine, because of its pulverulent form and the readiness with which it combines with the nitro-glycerine.

30 From this brief statement of the principles concerned it will be evident that there may be quite considerable variations both in proportions and in methods of operating without substantial change in the results produced. I will, however, give in detail the method which I consider best.

Having prepared and washed the nitro-glycerine, it is placed in a tank or "mixer," and to it are added the desired quantities of water and of the solid nitro-compound. The whole

is well mixed and stirred together. By from five to ten minutes' constant stirring a uniform mixture and pasty mass is produced which only requires packing in cartridges to fit it for use.

With regard to the quantity of the solid nitro-compound to be used, my rule is to add the solid to the liquid till the liquid mobility is removed. Where the cellulose compound has been well prepared, ten per cent. of it will accomplish the result. If, however, it be impure or ill prepared, it may still be used, but in somewhat larger quantity. The rule as given above I have found to meet all cases and to save much time and trouble.

The quantity of water to be used in this compound is difficult to state with exactitude, as the process allows of the mixture with the nitro-glycerine of any desired proportion of water. I have found, however, that where the mixing is thoroughly performed, the addition of two or three per cent. of water to one hundred per cent. of the freshly-washed nitro-glycerine is sufficient to confer practical safety.

Having now described my invention, I desire to disclaim as any part thereof the combination, broadly, of nitro-glycerine with any solid substances; but

What I do claim as new, and desire to secure by Letters Patent, is—

The method, substantially as described, for increasing the safety in handling or transportation of nitro-glycerine, consisting, essentially, in intimately mixing it with a pulverulent nitro-compound and water, as specified.

In witness whereof I have hereunto set my hand.

GILBERT S. DEAN.

Witnesses:

S. H. NOURSE,  
FRANK A. BROOKS.